# EUROPEAN PATENT SPECIFICATION

(11) **EP 3 884 016 B1**
(45) Date of publication and mention of the grant of the patent: **31.05.2023**
(21) Application number: 19835960.6
(22) Date of filing: 06.11.2019
(51) Int. Cl.: C10M 137/02, C10N 30/00, C10N 30/06, C10N 40/02, C10N 40/04

(54) **LUBRICATING COMPOSITION FOR AUTOMOTIVE OR INDUSTRIAL GEARS AND USE THEREOF**
SCHMIERMITTELZUSAMMENSETZUNG FÜR KRAFTFAHRZEUG- ODER INDUSTRIEGETRIEBE UND VERWENDUNG DERSELBEN
COMPOSITION LUBRIFIANTE POUR ENGRENAGE AUTOMOBILE OU INDUSTRIEL ET SON UTILISATION

(30) Priority: 12.11.2018 US 201862758729 P
(43) Date of publication of application: 29.09.2021
(62) Divisional of application: 23168061.2
(73) Proprietor: The Lubrizol Corporation, Wickliffe, Ohio 44092-2298 (US)
(72) Inventor: BARTON, William R.S., Belper Derbyshire DE56 1QN (GB)
(74) Representative: D Young & Co LLP
(86) International application number: PCT/US2019/060013
(87) International publication number: WO 2020/101969

(56) References cited:
- EP-A1- 0 686 690
- EP-A1- 2 025 739
- WO-A1-97/14770
- WO-A1-2017/079016

## Description

### BACKGROUND

The disclosed technology relates to a lubricant composition for automotive or industrial gears, as well as axles and bearings, the lubricant composition containing an oil of lubricating viscosity, a phosphate and/or thiophosphate compound, and a metal thiophosphate compound, such as zinc dialkyldithiophosphate, as well as use of the lubricant composition to improve automotive or industrial gear operating efficiency and temperature.

Driveline power transmitting devices (such as gears or transmissions) present highly challenging technological problems and solutions for satisfying the multiple and often conflicting lubricating requirements, while providing durability and cleanliness.

Improving operating efficiency is a common goal shared by both original equipment manufacturers and lubricant manufacturers. Original equipment manufacturers may focus on using mechanical processing methods to reduce surface roughness in an effort to improve operating efficiency. These mechanical processing methods include honing, top polishing, and vibratory finishing. Alternatively, lubricant manufacturers often target optimizing viscosity and lowering fluid traction coefficients in their efforts to optimize operating efficiency. Current mechanical processing methods can be expensive and time consuming to implement for large scale automotive gear production. Therefore, there is a desire to improve operating efficiency by modifying fluid properties, instead of relying on mechanical processes to achieve this goal.

EP 0686690 A1, granted Dec. 13, 1995, to Sanyo Chemical Ind. Ltd., discloses a gear or transmission lubricant composition, comprising a major portion of mineral base oil, containing added thereto (A) a phosphorus-containing metal-free organic compound, such as a phosphate ester or amine salt thereof, and (B) an oil-soluble copolymer of (a) an alkyl (meth)acrylate and (b) a N,N-dialkylaminoalkyl (meth)acrylate, for improved sludge dispersibility, in automatic transmission fluids.

WO 97/14770 A1, granted Apr. 24, 1997, to Exxon Chemical Patents Inc., discloses power transmitting fluids, particularly continuously variable transmission fluids, for improved antiwear performance incorporating an additive combination of amine phosphates, organic polysulfides, zinc salts of phosphorothioic acid esters and optionally a friction modifier.

US 10,316,712, granted Jun. 11, 2019 to Douglass et al., teaches the use of various additives to reduce the roughness of additive manufactured articles to maximize energy efficiency. The data in the '712 patent suggests that many different additives can function to reduce surface roughness, and in fact, that even an un-additized lubricant oil can reduce surface roughness. The '712 patent does not teach how to provide any other benefit to the lubricating oil, for example, such as providing the requisite performance in ASTM D7452, ASTM D6121, ASTM D4172 or ASTM D5704.

Therefore, a lubricant solution that can reduce surface roughness, reduce the fluid traction coefficient and/or improve fluid efficiency would be technically and commercially beneficial.

### SUMMARY

The use of amine alkyl(thio)phosphate chemistry with metal alkylthiophosphate chemistry not common to gear oil use was found to be beneficial for reducing surface roughness and improving traction coefficient, resulting in improving efficiency and reducing operation temperatures.

One aspect of the technology is directed to a lubricant composition comprising an oil of lubricating viscosity, from 0.5 to 2.0 wt% of an amine alkyl(thio)phosphate compound, and from 0.2 to 0.8 wt% of a metal alkylthiophosphate, wherein the lubricant comprises a total sulfur level of 2 to 5 wt%.

In embodiments, the amine alkyl(thio)phosphate can be simply an amine alkylphosphate. In other embodiments, the amine alkyl(thio)phosphate can be an amine alkylthiophosphate. In further embodiments, the amine alkyl(thio)phosphate can include a combination of both amine phosphate and amine alkylthiophosphate.

In an embodiment, the lubricant can include an amine phosphate that is a substantially sulfur-free alkyl phosphate amine salt having at least 30 mole percent of the phosphorus atoms in an alkyl pyrophosphate salt structure. In some embodiments, at least 80 mole percent of the alkyl groups in such a sulfur-free alkyl phosphate are secondary alkyl groups of 3 to 12 carbon atoms. In some embodiments, at least 25 mole percent of the alkyl groups in such a sulfur-free alkyl phosphate are primary alkyl groups of 3 to 12 carbon atoms.

In embodiments, the amine alkylthiophosphate can be a dialkyldithiophosphate.

The metal alkylthiophosphate in the lubricant composition can include a zinc dialkyldithiophosphate. In some embodiments, the zinc dialkyldithiophosphate can be a secondary zinc dialkyldithiophosphate.

The lubricant composition can also contain other additives. In an embodiment, the lubricant composition can include sulfur containing additives in an amount to provide the composition with a total sulfur level of 2 to 5 wt%. In an embodiment, the lubricant composition can have a total phosphorus level of 0.01 to 0.5 wt%.

Another aspect of the technology encompasses use of a lubricating composition for improving the operating temperatures of a gear at high load and low speed conditions, or the operating efficiency of a used gear, wherein the lubricant composition comprises: a. an oil of lubricating viscosity; b. 0.5 to 2.0 wt% of an amine alkyl(thio)phosphate compound, and c. 0.2 to 0.8 wt% of a metal alkylthiophosphate, wherein the lubricant comprises a total sulfur level of 2 to 5 wt%.

### DETAILED DESCRIPTION

Various preferred features and embodiments will be described below by way of non-limiting illustration. One aspect of the invention is a lubricant composition for a driveline device containing (a) an oil of lubricating viscosity, (b) at least one amine alkyl(thio)phosphate, and (b) a metal alkylthiophosphate as defined in the claims.

### Oil of Lubricating Viscosity

One component of the disclosed technology is an oil of lubricating viscosity, also referred to as a base oil. The base oil may be selected from any of the base oils in Groups I-V of the American Petroleum Institute (API) Base Oil Interchangeability Guidelines (2011), namely

| Base Oil Category | | Sulfur (%) | Saturates (%) | Viscosity Index |
|---|---|---|---|---|
| Group I | | >0.03 and/or | <90 | 80 to less than 120 |
| Group II | | ≤0.03 and | ≥90 | 80 to less than 120 |
| Group III | | ≤0.03 and | ≥90 | ≥120 |
| Group IV | All polyalphaolefins (PAOs) | | | |
| Group V | All others not included in Groups I, II, III or IV | | | |

Groups I, II and III are mineral oil base stocks. Other generally recognized categories of base oils may be used, even if not officially identified by the API: Group II+, referring to materials of Group II having a viscosity index of 110-119 and lower volatility than other Group II oils; and Group III+, referring to materials of Group III having a viscosity index greater than or equal to 130. The oil of lubricating viscosity can include natural or synthetic oils and mixtures thereof. Mixture of mineral oil and synthetic oils, e.g., polyalphaolefin oils and/or polyester oils, may be used.

In one embodiment the oil of lubricating viscosity has a kinematic viscosity at 100 °C by ASTM D445 of 1.5 to 7.5, or 2 to 7, or 2.5 to 6.5, or 3 to 6 mm²/s. In one embodiment the oil of lubricating viscosity comprises a poly alpha olefin having a kinematic viscotiy at 100 °C by ASTM D445 of 1.5 to 7.5 or any of the other aforementioned ranges.

### Amine Alkyl(Thio)Phosphates

The lubricant of the disclosed technology will include at least one amine alkyl(thio)phosphate. As used herein, the inclusion of "thio" in the parenthesis means that the phosphate may or may not contain sulfur atoms.

In one embodiment, the amine alkyl(thio)phosphate can include an amine phosphate, that is, a phosphate that is substantially sulfur-free. By substantially sulfur free it is meant that sulfur is not intentionally added to the amine phosphate, and preferably the amine phosphate is completely free of sulfur. However, it is recognized that in production situations some sulfur contamination may occur, resulting in some sulfur in the amine phosphate. To the extent the amine phosphate contains some sulfur contamination, such contaminated compound will still be considered to be substantially sulfur free if the sulfur does not affect the basic characteristics of the amine phosphate. Generally, sulfur contamination levels may be less than 2.5%, or 1%, 0.1%, or 0.01% by weight to be considered substantially sulfur free.

In an embodiment, the amine phosphate may include at least 30 mole percent of the phosphorus atoms in an alkyl pyrophosphate structure, as opposed to an orthophosphate (or monomeric phosphate) structure. The percentage of phosphorus atoms in the pyrophosphate structure may be 30 to 100 mole %, or 40 to 90 % or 50 to 80% or 55 to 70 % or 55 to 65%. The remaining amount of the phosphorus atoms may be in an orthophosphate structure or may consist, in part, in unreacted phosphorus acid or other phosphorus species. In one embodiment, up to 60 or up to 50 mole percent of the phosphorus atoms are in mono- or di-alkyl-orthophosphate salt structure.

In an embodiment, the amine phosphate, as present in the pyrophosphate form, may be represented in part by a half neutralized salt of formula (I) and/or a fully neutralized salt as in formula (II).

| | |
|---|---|
| | |
| (I) | (II) |

The extent of neutralization of the amine phosphate in practice, that is, the degree of salting of the -OH groups of the phosphorus esters, may be 50% to 100%, or 80% to 99%, or 90% to 98%, or 93% to 97%, or about 95%. Variants of these materials may also be present, such as a variant of formula (I) or formula (II) wherein the -OH group (in (I) is replaced by another -OR¹ group or wherein one or more -OR¹ groups are replaced by -OH groups, or wherein an R¹ group is replaced by a phosphorus-containing group, that is, those comprising a third phosphorus structure in place of a terminal R¹ group. Illustrative variant structures may include the following:

The structures of formulas (I) and (II) are shown as entirely sulfur-free species, in that the phosphorus atoms are bonded to oxygen, rather than sulfur atoms. However, it is possible that a small molar fraction of the O atoms could be replaced by S atoms, such as 0 to 5 percent or 0.1 to 4 percent or 0.2 to 3 percent or 0.5 to 2 percent.

The pyrophosphate salts may be distinguished from orthophosphate salts of the general structure which optionally may also be present in amounts as indicated above.

The amine phosphate may also include some amount of partial esters including mono- and diesters of the orthophosphate structure and diesters of the pyrophosphate structure.

In formulas (I) and (II), each R¹ is independently an alkyl group of 3 to 12 carbon atoms. The alkyl groups may be primary or secondary groups, or a mixture of both primary and secondary. In certain embodiments at least 80 mole percent, or at least 85, 90, 95, or 99 percent, of the R¹ alkyl groups will be secondary alkyl groups. In certain embodiments at least 25 mole percent, or at least 30, 40, 50, 60, 70, 80 or 90 or even 99 mole percent, of the R¹ alkyl groups will be primary alkyl groups.

In some embodiments the alkyl groups will have 3 or 4 to 12 carbon atoms, or 3 to 8, or 4 to 6, or 5 to 10, or 6 to 8 carbon atoms. The alkyl groups can be straight chain, branched or cyclic. Such groups include 2-butyl, 2-pentyl, 3-pentyl, 3-methyl-2-butyl, 2-hexyl, 3-hexyl, cyclohexyl, 4-methyl-2-pentyl, and other such secondary groups and isomers thereof having 6, 7, 8, 9, 10, 11, or 12 carbon atoms as well as propyl, butyl, isobutyl, pentyl, 3-methylbutyl, 2-methylbutyl, hexyl, heptyl, octyl, nonyl, decyl, undecyl, dodecyl, and other such primary groups and isomers thereof having 3, 4, 5, 6, 7, 8, 9, 10, 11, or 12 carbon atoms. In some embodiments the alkyl group will have a methyl branch at the α-position of the group, an example being the 4-methyl-2-pentyl (also referred to as 4-methylpent-2-yl) group.

The amine alkyl(thio)phosphate may also be an amine alkylthiophosphate, wherein the alkylthiophosphate is represented by the formula (R'O)₂PSSH, wherein each R' is independently a hydrocarbyl group containing from about 3 to about 30, preferably from about 3 up to about 18, or from about 3 up to about 12, or from up to about 8 carbon atoms. Example R' groups can include isopropyl, isobutyl, n-butyl, sec-butyl, the various amyl, n-hexyl, methylisobutyl carbinyl, heptyl, 2-ethylhexyl, isooctyl, nonyl, behenyl, decyl, dodecyl, and tridecyl groups. Illustrative lower alkylphenyl R' groups include butylphenyl, amylphenyl, heptylphenyl, etc. Examples of mixtures of R' groups include: 1-butyl and 1-octyl; 1-pentyl and 2-ethyl-1-hexyl; isobutyl and n-hexyl; isobutyl and isoamyl; 2-propyl and 2-methyl-4-pentyl; isopropyl and sec-butyl; and isopropyl and isooctyl.

In one embodiment, the alkylthiophosphate of the amine alkylthiophosphate may be reacted with an epoxide or a polyhydric alcohol, such as glycerol. This reaction product may be used alone, or further reacted with a phosphorus acid, anhydride, or lower ester. The epoxide is generally an aliphatic epoxide or a styrene oxide. Examples of useful epoxides include ethylene oxide, propylene oxide, butene oxide, octene oxide, dodecene oxide, styrene oxide, etc. Ethylene oxide and propylene oxide are preferred. The polyhydric alcohols are described above. The glycols may be aliphatic glycols having from 2 to about 12, or from about 2 to about 6, or from 2 or 3 carbon atoms. Glycols include ethylene glycol, propylene glycol, and the like. The alkylthiophosphate, glycols, epoxides, inorganic phosphorus reagents and methods of reacting the same are described in U.S. Pat. Nos. 3,197,405 and 3,544,465 .

Amine Component - The amine component of the amine alkyl(thio)phosphate may be represented by R²₃NH, where each R² is independently hydrogen or a hydrocarbyl group or an ester-containing group, or an ether-containing group, provided that at least one R² group is a hydrocarbyl group or an ester-containing group or an ether-containing group (that is, not NH₃). Suitable hydrocarbyl amines include primary amines having 1 to 18 carbon atoms, or 3 to 12, or 4 to 10 carbon atoms, such as methylamine, ethylamine, propylamine, isopropylamine, butylamine and isomers thereof, pentylamine and isomers thereof, hexylamine and isomers thereof, heptylamine and isomers thereof, octylamine and isomers thereof such as isooctylamine and 2-ethylhexylamine, as well as higher amines. Other primary amines include dodecylamine, fatty amines as n-octylamine, n-decylamine, n-dodecylamine, n-tetradecylamine, n-hexadecylamine, n-octadecylamine and oleylamine. Other useful fatty amines include commercially available fatty amines such as "Armeen^{®}" amines (products available from Akzo Chemicals, Chicago, Ill.), such as Armeen^{®} C, Armeen^{®} O, Armeen^{®} OL, Armeen^{®} T, Armeen^{®} HT, Armeen^{®} S and Armeen^{®} SD, wherein the letter designation relates to the fatty group, such as coco, oleyl, tallow, or stearyl groups.

Secondary amines that may be used include dimethylamine, diethylamine, dipropylamine, dibutylamine, diamylamine, dihexylamine, diheptylamine, methylethyl-amine, ethylbutylamine, bis-2-ethylhexylamine, N-methyl-1-amino-cyclohexane, Armeen^{®} 2C, and ethylamylamine. The secondary amines may be cyclic amines such as piperidine, piperazine and morpholine.

Suitable tertiary amines include tri-n-butylamine, tri-n-octylamine, tri-decylamine, tri-laurylamine, tri-hexadecylamine, and dimethyloleylamine (Armeen^{®} DMOD). Triisodecylamine or tridecylamine and isomers thereof may be used.

Examples of mixtures of amines include (i) an amine with 11 to 14 carbon atoms on tertiary alkyl primary groups, (ii) an amine with 14 to 18 carbon atoms on tertiary alkyl primary groups, or (iii) an amine with 18 to 22 carbon atoms on tertiary alkyl primary groups. Other examples of tertiary alkyl primary amines include tert-butylamine, tert-hexylamine, tert-octylamine (such as 1,1-dimethylhexylamine), tert-decylamine (such as 1,1-dimethyloctylamine), tertdodecylamine, tert-tetradecylamine, tert-hexadecylamine, tert-octadecylamine, tert-tetracosanylamine, and tert-octacosanyl-amine. In one embodiment a useful mixture of amines includes "Primene^{®} 81R" or "Primene^{®} JMT." Primene^{®} 81R and Primene^{®} JMT (both produced and sold by Rohm & Haas) may be mixtures of C11 to C14 tertiary alkyl primary amines and C18 to C22 tertiary alkyl primary amines, respectively.

In other embodiments the amine may be an ester-containing amine such as an N-hydrocarbyl-substituted γ- or δ-amino(thio)ester, which is therefore a secondary amine. The ester-containing amine, may, for example, be prepared by Michael addition of a primary amine, typically having a branched hydrocarbyl group, with an ethylenically unsaturated ester or thio ester, or, for example, by reductive amination of the esters of 5-oxy substituted carboxylic acids or 5-oxy substituted thiocarboxylic acids. They may also be prepared by amination of the esters of 5-halogen substituted carboxylic acids or 5-halogen substituted thiocarboxylic acids, or by reductive amination of the esters of 2-amino substituted hexanedioic acids, or by alkylation of the esters of 2-aminohexanedioic acids.

The amine, of whatever type, will be reacted to neutralize the acidic group(s) on the phosphorus ester component, to prepare the amine alkyl(thio)phosphate.

In an embodiment, the amine alkyl(thio)phosphate may be a phosphate amine of formulas (I) or (II), or variants thereof, with the amine being 2-ethylhexylamine.

In an embodiment, the amine alkyl(thio)phosphate may be an amine phosphate of formulas (I) or (II), or variants thereof, with the amine being an N-hydrocarbyl-substituted γ- or δ-amino(thio)ester.

In an embodiment, the alkylthiophosphate of the amine alkylthiophosphate comprises a dialkyldithiophosphate. In another embodiment, the amine of the amine alkylthiophosphate comprises a C₈ to C₂₀ alkylamine.

In one embodiment the amine alkyl(thio)phosphate can be an amine alkylthiophosphate that is the reaction product of a C₁₄ to C₁₈ alkylated dialkyldithiophosphoric acid with Primene 81R^{™} (produced and sold by Rohm & Haas) which is a mixture of C₁₁ to C₁₄ tertiary alkyl primary amines.

In embodiments, the amine alkyl(thio)phosphate can include combinations of amine phosphates, combinations of amine alkylthiophosphates, and combinations of amine phosphates with amine alkylthiophosphates.

The amount of amine alkyl(thio)phosphate in the lubricant composition is 0.5 to 2.0 percent, or 0.55 to 1.4 percent, or 0.6 to 1.3 percent, or 0.7 to 1.2, or 1 to 2, or even 1.5 to 2, or 1.2 to 1.8 percent by weight or even from 1.8 to 2.2 percent by weight. The amount may be suitable to provide phosphorus to the lubricant formulation in an amount of 200 to 3000 parts per million by weight (ppm), or 400 to 2000 ppm, or 300 to 2000, or 600 to 1500 ppm, or 700 to 1100 ppm, or 900 to 1900, or 1100 to 1800 ppm, or 1200 to 1600 ppm or 1500 to 2000 ppm.

It will be understood by the skilled person that the amine alkyl(thio)phosphate will typically comprise a mixture of various individual chemical species. Reference herein to an amine alkyl(thio)phosphate will be understood by those of ordinary skill to encompass mixtures of such compounds as may be prepared by the described syntheses.

### The Metal Alkylthiophosphate Compound

The lubricant composition will further include a metal alkylthiophosphate compound. The metal alkylthiophosphate compound can be represented by the formula: wherein R²⁵ and R²⁶ are independently hydrogen, hydrocarbyl groups or mixtures thereof, provided that at least one of R²⁵ and R²⁶ is a hydrocarbyl group, preferably an alkyl or cycloalkyl with 1 to 30, or 2 to 20 and in some cases 2 to 15 carbon atoms. In certain embodiments, R²⁵ and R²⁶ can be secondary alkyl groups of 2 to 8 carbon atoms, or even from 3 to 6 carbon atoms, such as, for example, those derived from 4-methylpentan-2-ol or isopropanol.

M is a metal, and n is an integer equal to the available valence of M. M is mono- or di- or trivalent, preferably divalent, more preferably a divalent transition metal, and most preferably zinc.

Examples of metal alkylthiophosphates include zinc isopropyl methyl-amyl dithiophosphate, zinc isopropyl isooctyl dithiophosphate, zinc di(cyclohexyl)dithiophosphate, zinc isobutyl 2-ethylhexyl dithiophosphate, zinc isopropyl 2-ethylhexyl dithiophosphate, zinc isobutyl isoamyl dithiophosphate, zinc isopropyl n-butyl dithiophosphate, calcium di(hexyl)dithiophosphate, barium di(nonyl)dithiophosphate, zinc di(isobutyl) dithiophosphate, zinc isopropyl secondary-butyl dithiophosphate, zinc isopropyl dithiophosphate, zinc isopropyl 4-methylpentan-2-ol dithiophosphate, zinc 4-methylpentan-2-ol dithiophosphate or mixtures thereof.

The metal alkylthiophosphate may be a zinc dialkyldithiophosphate. Zinc dialkyldithiophosphates may be described as primary zinc dialkyldithiophosphates or as secondary zinc dialkyldithiophosphates, depending on the structure of the alcohol used in its preparation. In some embodiments the lubricant composition can include a primary zinc dialkyldithiophosphate. In some embodiments the lubricant composition can include a secondary zinc dialkyldithiophosphate. In some embodiments the lubricant composition can include a mixture of primary and secondary zinc dialkyldithiophosphates.

Metal from the metal alkylthiophosphate, such as zinc, may be supplied at a concentration of from 0.02 to 0.095 wt% zinc, or from 0.025 to 0.085 wt%, or even from 0.03 to 0.075 wt% zinc. Such levels may be associated with a metal alkylthiophosphate concentration of from 0.2 to 0.8 wt%, of from 0.25 to 0.75 wt%, or even from 0.3 to 0.70 wt%

In embodiments, the metal alkylthiophosphate can provide from 0.01 or from 0.02 to about 0.095 wt% phosphorus, or from about 0.025 to 0.085 wt%, or even from about 0.03 to about 0.075 wt% phosphorus.

In embodiments, the metal alkylthiophosphate can provide from 0.01 or from 0.02 to about 0.2 wt% phosphorus, or from about 0.025 to 0.19 wt%, or even from about 0.03 to about 0.18 wt% phosphorus.

### Other Additives

The lubricant composition can also contain other sulfur containing compounds, such as, for example, organo-sulfides, including polysulfides, such as sulfurized olefins, thiadiazoles and thiadiazole adducts such as post treated dispersants.

The organo-sulfide can be present in a range of 0 wt % to 6 wt %, 4 wt % to 6 wt %, 0.5 wt % to 3 wt %, 3 wt % to 5 wt %, 0 wt % to 1 wt %, 0.1 wt % to 0.5 wt %, 1% to 3%, 2% to 3%, 3% to 4%, or 2% to 4% of the lubricating composition.

The organosulfide may alternatively be a polysulfide. In one embodiment at least about 50 wt % of the polysulfide molecules are a mixture of tri- or tetra-sulfides. In other embodiments at least about 55 wt %, or at least about 60 wt % of the polysulfide molecules are a mixture of tri- or tetra-sulfides. The polysulfides include sulfurized organic polysulfides from oils, fatty acids or ester, olefins or polyolefins.

Oils which may be sulfurized include natural or synthetic oils such as mineral oils, lard oil, carboxylate esters derived from aliphatic alcohols and fatty acids or aliphatic carboxylic acids (e.g., myristyl oleate and oleyl oleate), and synthetic unsaturated esters or glycerides.

Fatty acids include those that contain 8 to 30, or 12 to 24 carbon atoms. Examples of fatty acids include oleic, linoleic, linolenic, and tall oil. Sulfurized fatty acid esters prepared from mixed unsaturated fatty acid esters such as are obtained from animal fats and vegetable oils, including tall oil, linseed oil, soybean oil, rapeseed oil, and fish oil.

The polysulfide may also be derived from an olefin derived from a wide range of alkenes, typically having one or more double bonds. The olefins in one embodiment contain 3 to 30 carbon atoms. In other embodiments, olefins contain 3 to 16, or 3 to 9 carbon atoms. In one embodiment the sulfurized olefin includes an olefin derived from propylene, isobutylene, pentene, or mixtures thereof. In one embodiment the polysulfide comprises a polyolefin derived from polymerizing, by known techniques, an olefin as described above. In one embodiment the polysulfide includes dibutyl tetrasulfide, sulfurized methyl ester of oleic acid, sulfurized alkylphenol, sulfurized dipentene, sulfurized dicyclopentadiene, sulfurized terpene, and sulfurized Diels-Alder adducts; phosphosulfurized hydrocarbons.

Examples of a thiadiazole include 2,5-dimercapto-1,3,4-thiadiazole, or oligomers thereof, a hydrocarbyl-substituted 2,5-dimercapto-1,3-4-thiadiazole, a hydrocarbylthio-substituted 2,5-dimercapto-1,3-4-thiadiazole, or oligomers thereof. The oligomers of hydrocarbyl-substituted 2,5-dimercapto-1,3-4-thiadiazole typically form by forming a sulfur-sulfur bond between 2,5-dimercapto-1,3-4-thiadiazole units to form oligomers of two or more of said thiadiazole units. Further examples of thiadiazole compounds are found in WO 2008,094759, paragraphs 0088 through 0090.

Described herein is a method of more substantially reducing friction/traction and the roughness of a metal surface. The method includes placing the metal surface under boundary or mixed lubrication conditions in the presence of the lubricant, that is, providing to the metal surface the lubricant composition as described herein. The term "boundary or mixed conditions" means operating conditions under which the metal surface of a device is in such proximity to another surface that some physical contact between asperities on the metal surface and asperities on the other surface is possible during operation of the device. Thus, by "placing the metal surface under boundary or mixed lubrication conditions" it is meant that the metal surface of a device is subject to boundary or mixed conditions with another surface and the device is operated such that the boundary conditions exist. An example of placing a metal surface under boundary conditions includes the operation of a gear on a driveline device, in which the gears are in such close proximity that some physical contact of the gear surfaces is possible.

The technology also provides use of a lubricant composition, as defined herein, to improve the operating temperatures of a gear at high load and low speed conditions.

The technology also provides use of a lubricant composition, as defined herein, to improving the operating efficiency of a used gear. By "used gear" it means a gear that has been in operation in it intended application. For example, an automotive gear employed in the operation of an automotive vehicle would be considered a used gear, or an industrial gear employed in its industrial application would be considered a used gear.

In particular, described herein is a method of lubricating a driveline device, comprising supplying thereto a lubricant composition as described herein, that is, a lubricant composition containing (a) an oil of lubricating viscosity and (c) a metal alkylthiophosphate, or in some instance, (a) an oil of lubricating viscosity, (b) an amine alkyl(thio)phosphate, and (c) a metal alkylthiophosphate, and operating the driveline device for a sufficient period to allow the lubricant composition to reduce the friction/traction and roughness of metal surfaces on the driveline device in a controlled manner to a greater extent than a typical gear lubricant. This reduction in surface roughness can be visually observed, or deduced in other ways, such as by a measured reduction in traction coefficient between two metal surfaces in the device, or by efficiency measurements on the driveline device before and after operation with the lubricant composition.

The driveline device may comprise a gear as in a gearbox of a vehicle (e.g., a manual transmission) or in an axle or differential, or in other driveline power transmitting driveline devices. The driveline device may also include bearings. Lubricated gears may include hypoid gears, such as those for example in a rear drive axle.

The lubricant should be able to meet the other aspects expected of it in normal operation of the driveline device.

As used herein, the term "condensation product" is intended to encompass esters, amides, imides and other such materials that may be prepared by a condensation reaction of an acid or a reactive equivalent of an acid (e.g., an acid halide, anhydride, or ester) with an alcohol or amine, irrespective of whether a condensation reaction is actually performed to lead directly to the product. Thus, for example, a particular ester may be prepared by a transesterification reaction rather than directly by a condensation reaction. The resulting product is still considered a condensation product.

The amount of each chemical component described is presented exclusive of any solvent or diluent oil, which may be customarily present in the commercial material, that is, on an active chemical basis, unless otherwise indicated. However, unless otherwise indicated, each chemical or composition referred to herein should be interpreted as being a commercial grade material which may contain the isomers, by-products, derivatives, and other such materials which are normally understood to be present in the commercial grade.

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having predominantly hydrocarbon character. Examples of hydrocarbyl groups include:
- hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form a ring);
- substituted hydrocarbon substituents, that is, substituents containing non-hydrocarbon groups which, in the context of this invention, do not alter the predominantly hydrocarbon nature of the substituent (e.g., halo (especially chloro and fluoro), hydroxy, alkoxy, mercapto, alkylmercapto, nitro, nitroso, and sulfoxy);
- hetero substituents, that is, substituents which, while having a predominantly hydrocarbon character, in the context of this invention, contain other than carbon in a ring or chain otherwise composed of carbon atoms and encompass substituents as pyridyl, furyl, thienyl and imidazolyl. Heteroatoms include sulfur, oxygen, and nitrogen. In general, no more than two, or no more than one, non-hydrocarbon substituent will be present for every ten carbon atoms in the hydrocarbyl group; alternatively, there may be no non-hydrocarbon substituents in the hydrocarbyl group.

It is known that some of the materials described herein may interact in the final formulation, so that the components of the final formulation may be different from those that are initially added. For instance, metal ions (of, e.g., a detergent) can migrate to other acidic or anionic sites of other molecules. The products formed thereby, including the products formed upon employing the composition of the present invention in its intended use, may not be susceptible of easy description. Nevertheless, all such modifications and reaction products are included within the scope of the present invention; the present invention encompasses the composition prepared by admixing the components described above.

The invention herein may be better understood with reference to the following examples.

### EXAMPLES

Three fluids were evaluated in a bench screen test procedure developed and conducted by Wedeven Associates on a WAM ball-on-disc test machine. A commercially available 80W-90 fluid and two additional fluids formulated as 75W-85 oils were evaluated. Samples 1 (not according to the invention) and 2 (inventive) were prepared according to the recipe in Table 1 Testing was completed under ambient conditions with a changing speed profile to allow gradual reduction in the lubricant film from hydrodynamic to boundary. A single stress (160ksi) was maintained over the range of speeds. Traction coefficients were measured for each fluid in duplicate over seven stages.

**Table 1. - Sample formulations 1-2.**

| | Sample 1 | Sample 2 |
|---|---|---|
| Synthetic basestock | 75.4 | 75.4 |
| Olefin copolymer | 14.6 | 14.6 |
| Succinimide dispersant | 1.32 | 1.32 |
| Substituted thiadiazole | 0.6 | 0.6 |
| Phosphoric acid ester/amine salt | 1.2 | 1.2 |
| Dialkyl hydrogen phosphate | 0.2 | 0.2 |
| Substituted triazole | 0.05 | 0.05 |
| Sulfurized olefin A | 4.5 | |
| Sulfurized olefin B | | 4.5 |
| Secondary ZDDP | | 0.31 |
| Glycerol ester | | 0.2 |
| KV at 40°C | 65.48 | 60.89 |
| KV at 100°C | 11.53 | 10.95 |
| VI | 172 | 174 |
| P, ppm | 1210 | 1474 |
| S, ppm | 21080 | 24830 |
| Zn, ppm | | 377 |

Test conditions were:
Ball: Carburised 4320, Ra 13 µ-inch
Disc: Carburised 4320, Ra 15 µ-inch
Entraining velocity per stage, 7 stages per cycle: 9, 5, 2.5, 0.6, 0.1, 0.06, 0.6 m/sec
Run time for each cycle: 3200 seconds
Slip/skew: 75%/41°
Stress: 160 ksi

All tests were run in duplicate and the average of the two runs is reported in the table below. The reduction in entraining velocity from stage 1 to stage 6 takes the lubrication regime from hydrodynamic to boundary. As the entraining velocity decreases, the oil film thickness decreases, the asperity interaction increases, and the traction coefficient increases to a maximum in stage 6. In stage 7, the entrainment velocity increases to be identical to stage 4. The relative difference in traction between these conditions is one indicator that surface modification and roughness reduction has been achieved during stages 5 and 6 which are intended to operate in mixed and boundary contact. A reduction in traction coefficient from stage 4 to 7 is expected if roughness has been reduced.

**Table 2. Traction coefficients**

| | Stage 1 | Stage 2 | Stage 3 | Stage 4 | Stage 5 | Stage 6 | Stage 7 |
|---|---|---|---|---|---|---|---|
| Commercial | 0.029 | 0.04 | 0.057 | 0.097 | 0.107 | 0.109 | 0.094 |
| Sample 1 | 0.057 | 0.075 | 0.09 | 0.101 | 0.106 | 0.109 | 0.1 |
| Sample 2 | 0.043 | 0.051 | 0.064 | 0.09 | 0.112 | 0.127 | 0.083 |

Roughness measurements were made at three locations for each run (6 measurements were recorded in total as each fluid was run twice) both within and outside of the contact zone. From these measurements an average % change was calculated inside the contact zone vs outside the contact zone. The averages are reported in the table below. The largest roughness reduction was recorded for Sample 2 containing the ZDDP.

**Table 3. Roughness reduction**

| | Ball | Disc |
|---|---|---|
| Commercial | 11 | 22 |
| Sample 1 | 32 | 24 |
| Sample 2 | 53 | 49 |

Because the viscosity grade for the commercial sample is not the same as the viscosity grades of Samples 1 and 2, and there were multiple formulation changes made between samples 1 and 2, additional work was carried out to help pinpoint what the main cause of the observed results could be attributed to. Samples 3 through 5 (not according to the invention) and 6 (inventive) were prepared to help isolate some of the differences between fluids 1 and 2 and to determine if the nature of the phosphorus ester amine salt would have an impact on the traction coefficient. The formulations were simplified compared to Samples 1 and 2 and all fluids were formulated to have a target kinematic viscosity of 5.9cSt.

**Table 4. Fluid formulations for samples 3-6.**

| | Sample 3 | Sample 4 | Sample 5 | Sample 6 |
|---|---|---|---|---|
| Synthetic base stock | 82.1 | 82.1 | 82.1 | 82.1 |
| 100cSt PAO | 12 | 12 | 12 | 12 |
| Sulfurized olefin | 4.3 | 4.3 | 4.3 | 4.3 |
| Substituted thiadiazole | 0.2 | 0.2 | 0.2 | 0.2 |
| S-free phos ester amine salt | 1.4 | 0.7 | 0.7 | 0.7 |
| S-containing phos ester amine salt | | 0.7 | 0.7 | |
| Glycerol ester | | | 2 | |
| Low molecular weight secondary ZDDP | | | | 0.6 |
| KV at 40°C | 28.66 | 28.83 | 29.54 | 28.63 |
| KV at 100°C | 5.899 | 5.916 | 5.969 | 5.887 |
| VI | 156 | 156 | 153 | 156 |
| P, ppm | 1173 | 1223 | 1228 | 1256 |
| S, ppm | 19768 | 20935 | 20446 | 21046 |
| Zn, ppm | | | | 707 |

Samples 3-6 were evaluated on the WAM ball-on-disc test machine under identical conditions to those outlined for samples 1 and 2. While samples 1 and 2 were evaluated after only one cycle, samples 3 - 6 were evaluated by repeating the seven-stage procedure six times. Traction measurements were made at each stage and roughness measurements were made both within the contact zone and outside of the contact zone after all six cycles were completed. Traction measurements are recorded in the table below over all seven stages for both the first and the last cycle.

**Table 5. Traction coefficients for samples 3-6.**

| | | Stage 1 | Stage 2 | Stage 3 | Stage 4 | Stage 5 | Stage 6 | Stage 7 |
|---|---|---|---|---|---|---|---|---|
| Sample 3 | Cycle 1 | 0.082 | 0.088 | 0.096 | 0.107 | 0.11 | 0.113 | 0.105 |
| | Cycle 6 | 0.053 | 0.069 | 0.087 | 0.104 | 0.108 | 0.111 | 0.102 |
| | % Change | -36 | -22 | -10 | -3 | -2 | -2 | -3 |
| Sample 4 | Cycle 1 | 0.07 | 0.072 | 0.093 | 0.108 | 0.113 | 0.115 | 0.107 |
| | Cycle 6 | 0.05 | 0.066 | 0.085 | 0.102 | 0.106 | 0.111 | 0.102 |
| | % Change | -29 | -9 | -9 | -6 | -6 | -3 | -5 |
| Sample 5 | Cycle 1 | 0.085 | 0.082 | 0.092 | 0.102 | 0.104 | 0.105 | 0.101 |
| | Cycle 6 | 0.048 | 0.069 | 0.085 | 0.1 | 0.104 | 0.105 | 0.1 |
| | % Change | -44 | -16 | -8 | -2 | 0 | 0 | -1 |
| Sample 6 | Cycle 1 | 0.067 | 0.066 | 0.069 | 0.093 | 0.11 | 0.126 | 0.088 |
| | Cycle 6 | 0.025 | 0.034 | 0.045 | 0.066 | 0.084 | 0.109 | 0.064 |
| | % Change | -62 | -49 | -35 | -29 | -23 | -13 | -28 |

Comparisons can be made for each fluid between cycle 1 data at a given stage and cycle 6 data at the same stage also, this describes the repeated roughness reduction from the lubricant over more cycles. The % change reported in the table represents this change in traction coefficient between cycle 1 and 6 and again shows sample 6 to be superior to samples 3-5. The addition of friction modifier has little influence on the traction results of sample 5 compared to sample 4.

Roughness reduction can be observed visually and measured/reported as a roughness change after 6 cycles. Table 6 below indicates the change in roughness of both the ball and the disc from beginning to the end of the test. Results reported in the table represent an average of six measurements made on the ball and disc parts. The greatest reduction in roughness is observed for sample 6.

**Table 6. - Roughness change after six cycles.**

| | Ball | Disc |
|---|---|---|
| Sample 3 | 21 | 37 |
| Sample 4 | 36 | 30 |
| Sample 5 | 34 | 30 |
| Sample 6 | 59 | 42 |

Additional traction data was gathered for Samples 7-10. Samples 7 (not according to the invention) and 8 (inventive) are identical, except that sample 8 contains both a S-containing phos ester amine salt and ZDDP. Samples 9 (not according to the invention) and 10 (inventive) are identical to each other, but Sample 10 contains both a S-free phos ester amine salt and ZDDP. These samples were analyzed using a standard mini-traction machine (MTM). A frictional force of 1.0GPa pressure was applied at a temperature of 140°C at a mean speed of 100 mm/s and 250% slide-to-roll ratio (SRR).

**Table 7. Fluid formulations for samples 7 - 10.**

| | Sample 7 | Sample 8 | Sample 9 | Sample 10 |
|---|---|---|---|---|
| Olefin copolymer | 14.6 | 14.6 | 14.6 | 14.6 |
| Sulfurized olefin | 4.5 | 4.5 | 4.5 | 4.5 |
| Succinimide dispersant | 1.32 | 1.32 | 1.32 | 1.32 |
| Substituted thiadiazole | 0.6 | 0.6 | 0.6 | 0.6 |
| Glycerol ester | 0.2 | 0.2 | 0.2 | 0.2 |
| S-containing phos ester amine salt | 1.2 | 1.2 | | |
| S-free phos ester amine salt | | | 1.2 | 1.2 |
| Low molecular weight secondary ZDDP | | 0.31 | | 0.31 |
| Oil of lubricating viscosity | Sum to 100 | Sum to 100 | Sum to 100 | Sum to 100 |
| P, ppm | 1336 | 1013 | 1006 | 1241 |
| S, ppm | 22300 | 21500 | 20700 | 20800 |
| Zn, ppm | 369 | | | 336 |

Traction coefficients were recorded over time. A subset of the data is reported in the table below. Note that early in the test, traction coefficients for all fluids are relatively similar, however, over longer time periods, the results begin to diverge. Samples 8 and 10 containing ZDDP show a large reduction in traction coefficient over time, while the traction coefficients of Samples 7 and 9 stay relatively constant over the course of the entire test.

**Table 8. Traction coefficient data for samples 7-10 measured in MTM rig.**

| Time (s) | Sample 7 | Sample 8 | Sample 9 | Sample 10 |
|---|---|---|---|---|
| 250 | 0.1506 | 0.1563 | 0.1397 | 0.1449 |
| 500 | 0.1481 | 0.1581 | 0.1415 | 0.1467 |
| 1000 | 0.1499 | 0.1581 | 0.1417 | 0.1495 |
| 2000 | 0.1509 | 0.1523 | 0.1399 | 0.1445 |
| | | | | |
| 12250 | 0.1465 | 0.0595 | 0.1373 | 0.1062 |
| 12500 | 0.1473 | 0.0582 | 0.138 | 0.106 |
| 13000 | 0.1485 | 0.0576 | 0.1379 | 0.104 |
| 14000 | 0.1506 | 0.0552 | 0.1373 | 0.1029 |

While the stressing conditions that the oils were subjected to were very different in the Wedeven testing vs. the MTM testing, the outcome was the same. Under both sets of conditions, fluids containing both an amine phosphate and a ZDDP demonstrated lower traction coefficients over time compared to fluids containing only an amine phosphate.

At Wedeven, axle efficiency for Sample 2 was measured on a used axle (medium duty axle with 25000 miles service). Testing included running steady state conditions before and after a conditioning period consisting of extended speed-load cycling. Steady state conditions consisted of one temperature (80C) at high and low pinion speeds and five loads (pinion torque). The gear conditioning period was divided into two stages. The first stage was conducted at 79°C, while the second stage was conducted at 93°C. Each stage was run at 11 different pinion speeds (approximately 250-3000 RPM) and seven different pinion torques (approximately 50-200 lb-ft). These extended speed and load conditions allow reduced friction on the already broken-in-axle if the lubricant were capable of further reducing surface roughness. The pre-extended phase and post extended phase comparisons are shown in the table below. Across all conditions with the exception of the lowest load, higher speed condition, there is a marked benefit to operating efficiency after the extended speed-load procedure. The gains are significant in an already efficient operating environment and indicate that despite significant use in the field, the lubricant was able to further improve efficiency by a further reduction in surface roughness during the conditioning phase.

**Table 9. - Efficiency change.**

| Pinion Speed | Pinion Power | Efficiency (pre) | Efficiency (post) | Efficiency Change |
|---|---|---|---|---|
| rpm | kW | (%) | (%) | (%) |
| High | 13.1 | 85.23 | 85.14 | -0.09 |
| | 26.2 | 90.92 | 91.14 | 0.22 |
| | 52.4 | 93.55 | 94.08 | 0.53 |
| | 78.6 | 94.24 | 94.95 | 0.71 |
| Low | 3.7 | 88.25 | 89.17 | 0.92 |
| | 7.3 | 90.94 | 91.96 | 1.02 |
| | 14.7 | 92.15 | 93.21 | 1.06 |
| | 22.0 | 92.5 | 93.5 | 1 |
| | 29.3 | 92.72 | 93.58 | 0.86 |

The table below shows the roughness measurements of select ring and pinion teeth with Sample 2, confirming that a reduction in tooth roughness on an already used axle has been achieved. Combined with the efficiency data this demonstrates efficiency benefits can be achieved in existing hardware without the need for expensive surface finishing or radically low fluid viscosities.

**Table 10. - Roughness change.**

| Roughness, Ra (µin) | | | | |
|---|---|---|---|---|
| | Tooth | Before | After | % Change |
| Pinion | 1 | 22.9 | 21.5 | 6.1 |
| | 3 | 27.9 | 21.6 | 22.6 |
| | 4 | 21.8 | 16.1 | 26.1 |
| | 5 | 26.8 | 18.1 | 32.5 |
| | Avg. | 24.9 | 19.3 | 22.2 |
| Ring | 7 | 19.0 | 13.2 | 30.5 |
| | 9 | 16.7 | 13.4 | 19.8 |
| | 10 | 25.2 | 23.1 | 8.3 |
| | Avg | 20.3 | 16.6 | 18.4 |

In addition to the operating efficiency benefits in torque loss measurements, gear oil fluids containing ZDDP can also improve operating temperatures at high load, low speed conditions. A modified L-37 test was developed with controlled air flow instead of cooling water during the test phase. This allowed the test temperature to fluctuate as it would in operation rather than operate in a controlled manner as is typical of industry testing.

The procedure was run on Dana 60 hardware approved for L-37 testing in a 2-phase test based on the standard L-37 procedure, ASTM D6121-16a. Setup deviations include filling the axle to exactly 3 liters to allow for some oil to be lost during ancillary test phase drains, and using a modified axle cover to allow operations to do purges, refills and drains during test. Conditioning parameters match with ASTM D6121 L-37 specification including loads, speeds and temperature control.

The test phase, or phase 2, is modified from standard practice in D6121. In place of spray-water temperature control and a temperature setpoint, the axle sump temperature direct control is removed, allowing the axle to float to any temperature below the operator safety shutoff of 190 °C. The axle is kept from reaching excessive temperatures by a constant velocity and trajectory of controlled air pushed over the axle and through the enclosure at 7.11 meters/second through an entry duct above the center housing with diameter of 15.24 centimeters. Furthermore, load is set to 13% contact stress reduction load setpoints specified in D6121-16a section A9.4 (1645Nm +- 34Nm) using a non-load-reduced axle batch to help further decrease risk of exceeding temperature limits without cooling water control. All other parameters and standards of this phase of the procedure are in accordance with relevant sections of ASTM D6121-16a.

**Table 11. Fluid formulations for samples 11 (not according to the invention) - 12 (inventive).**

| | Sample 11 | Sample 12 |
|---|---|---|
| Alkyl ester polymer | 12.4 | 12.4 |
| Sulfurized olefin | 4.6 | 4.6 |
| Borated dispersant | 0.78 | 0.78 |
| Substituted thiadiazole | 0.15 | 0.15 |
| Alkyl amide | 0.13 | 0.13 |
| Antifoam | 0.1 | 0.1 |
| Corrosion inhibitor | 0.04 | 0.04 |
| Phosphate ester amine | 1.66 | 1.46 |
| Low molecular weight secondary ZDDP | | 0.3 |
| Oil of lubricating viscosity | Sum to 100 | Sum to 100 |
| P, ppm | 1431 | 1484 |
| S, ppm | 20800 | 22300 |
| Zn, ppm | | 367 |

Table 12 below shows the results of these evaluations and confirms that use of ZDDP in a gear oil fluid results in a substantial decrease in operating temperature in the modified L-37 test. Both fluids show exceptional wear performance.

**Table 12. Operating temperatures in modified L-37 testing for samples 11 - 12.**

| | Peak Temp | Final Temp | Pinion/ring wear |
|---|---|---|---|
| Sample 11 | 164.9 | 115 | 8/9 |
| Sample 12 | 144.4 | 110 | 9/9 |

The mention of any document is not an admission that such document qualifies as prior art or constitutes the general knowledge of the skilled person in any jurisdiction. It is to be understood that the upper and lower amount, range, and ratio limits set forth herein may be independently combined. Similarly, the ranges and amounts for each element of the invention can be used together with ranges or amounts for any of the other elements.

As used herein, the transitional term "comprising," which is synonymous with "including," "containing," or "characterized by," is inclusive or open-ended and does not exclude additional, un-recited elements or method steps. However, in each recitation of "comprising" herein, it is intended that the term also encompass, as alternative embodiments, the phrases "consisting essentially of' and "consisting of," where "consisting of" excludes any element or step not specified and "consisting essentially of" permits the inclusion of additional un-recited elements or steps that do not materially affect the essential or basic and novel characteristics of the composition or method under consideration. The expression "consisting of" or "consisting essentially of," when applied to an element of a claim, is intended to restrict all species of the type represented by that element, notwithstanding the presence of "comprising" elsewhere in the claim.

While certain representative embodiments and details have been shown for the purpose of illustrating the subject invention, it will be apparent to those skilled in this art that various changes and modifications can be made therein without departing from the scope of the subject invention. In this regard, the scope of the invention is to be limited only by the following claims.

## Claims

1. A lubricant composition comprising
a. an oil of lubricating viscosity;
b. 0.5 to 2.0 wt% of an amine alkyl(thio)phosphate compound, and
c. 0.2 to 0.8 wt% of a metal alkylthiophosphate,
wherein the lubricant composition comprises a total sulfur level of 2 to 5 wt%.

2. The lubricant composition of claim 1, wherein the amine alkyl(thio)phosphate comprises an amine phosphate.

3. The lubricant composition of claim 2, where the amine phosphate comprises a substantially sulfur-free alkyl phosphate amine salt wherein at least 30 mole percent of the phosphorus atoms are in an alkyl pyrophosphate salt structure and at least 80 mole percent of the alkyl groups are secondary alkyl groups of 3 to 12 carbon atoms; or where the amine phosphate comprises a substantially sulfur-free alkyl phosphate amine salt wherein at least 30 mole percent of the phosphorus atoms are in an alkyl pyrophosphate salt structure and at least 25 mole percent of the alkyl groups in such a sulfur-free alkyl phosphate are primary alkyl groups of 3 to 12 carbon atoms.

4. The lubricant composition of any previous claim wherein the amine comprises 2-ethylhexylamine.

5. The lubricant composition of any previous claim wherein the amine comprises an N-hydrocarbyl-substituted γ- or δ-amino(thio)ester.

6. The lubricant composition of claim 1 or 2, wherein the amine alkyl(thio)phosphate comprises an amine alkylthiophosphate.

7. The lubricant composition of claim 6, wherein the alkylthiophosphate of the amine alkylthiophosphate comprises a dialkyldithiophosphate.

8. The lubricant composition of claim 6 or 7, wherein the amine comprises a C₈ to C₂₀ alkylamine.

9. The lubricant composition of any previous claim, wherein the metal alkylthiophosphate comprises zinc dialkyldithiophosphate.

10. The lubricant composition of claim 9, wherein the zinc dialkyldithiophosphate comprises, consists essentially of, or consists of a secondary zinc dialkyldithiophosphate, preferably wherein the alkyl of the zinc dialkyldithiophosphate comprises 3 to 6 carbon atoms.

11. The lubricant composition of claim 9 or 10, wherein the zinc dialkyldithiophosphate provides from 0.02 to 0.095 wt% zinc to the lubricant composition.

12. The lubricant composition of any previous claim further comprising less than 6 wt% of an organo-sulfide, preferably wherein the organo-sulfide comprises 2,5-dimercapto-1,3,4-thiadiazole.

13. Use of a lubricating composition for improving the operating temperatures of a gear at high load and low speed conditions, or the operating efficiency of a used gear, wherein the lubricant composition comprises:
a. an oil of lubricating viscosity;
b. 0.5 to 2.0 wt% of an amine alkyl(thio)phosphate compound, and
c. 0.2 to 0.8 wt% of a metal alkylthiophosphate, wherein the lubricant comprises a total sulfur level of 2 to 5 wt%.

## Patentansprüche

1. Schmiermittelzusammensetzung, umfassend
a. ein Öl mit Schmierviskosität;
b. zu 0,5 bis 2,0 Gew.-% eine Aminalkyl(thio)phosphatverbindung und
c. zu 0,2 bis 0,8 Gew.-% ein Metallalkylthiophosphat,
wobei die Schmiermittelzusammensetzung einen Gesamtschwefelgehalt von 2 bis 5 Gew.-% umfasst.

2. Schmiermittelzusammensetzung nach Anspruch 1, wobei das Aminalkyl(thio)phosphat ein Aminphosphat umfasst.

3. Schmiermittelzusammensetzung nach Anspruch 2, wobei das Aminphosphat ein im Wesentlichen schwefelfreies Alkylphosphataminsalz umfasst, wobei mindestens 30 Molprozent der Phosphoratome in einer Alkylpyrophosphatsalz-Struktur liegen und mindestens 80 Molprozent der Alkylgruppen sekundäre Alkylgruppen von 3 bis 12 Kohlenstoffatomen sind; oder wobei das Aminphosphat ein im Wesentlichen schwefelfreies Alkylphosphataminsalz umfasst, wobei mindestens 30 Molprozent der Phosphoratome in einer Alkylpyrophosphatsalz-Struktur liegen und mindestens 25 Molprozent der Alkylgruppen in einem solchen schwefelfreien Alkylphosphat primäre Alkylgruppen von 3 bis 12 Kohlenstoffatomen sind.

4. Schmiermittelzusammensetzung nach einem der vorstehenden Ansprüche, wobei das Amin 2-Ethylhexylamin umfasst.

5. Schmiermittelzusammensetzung nach einem der vorstehenden Ansprüche, wobei das Amin einen N-Hydrocarbyl-substituierten γ- oder δ-Amino(thio)ester umfasst.

6. Schmiermittelzusammensetzung nach Anspruch 1 oder 2, wobei das Aminalkyl(thio)phosphat ein Aminalkylthiophosphat umfasst.

7. Schmiermittelzusammensetzung nach Anspruch 6, wobei das Alkylthiophosphat des Aminalkylthiophosphats ein Dialkyldithiophosphat umfasst.

8. Schmiermittelzusammensetzung nach Anspruch 6 oder 7, wobei das Amin ein C₈ bis C₂₀-Alkylamin umfasst.

9. Schmiermittelzusammensetzung nach einem der vorstehenden Ansprüche, wobei das Metallalkylthiophosphat Zinkdialkyldithiophosphat umfasst.

10. Schmiermittelzusammensetzung nach Anspruch 9, wobei das Zinkdialkyldithiophosphat ein sekundäres Zinkdialkyldithiophosphat umfasst, im Grunde daraus besteht oder daraus besteht, vorzugsweise wobei das Alkyl des Zinkdialkyldithiophosphats 3 bis 6 Kohlenstoffatome umfasst.

11. Schmiermittelzusammensetzung nach Anspruch 9 oder 10, wobei das Zinkdialkyldithiophosphat von 0,02 bis 0,095 Gew.-% Zink zu der Schmiermittelzusammensetzung bereitstellt.

12. Schmiermittelzusammensetzung nach einem der vorstehenden Ansprüche, ferner umfassend zu weniger als 6 Gew.-% ein Organosulfid, vorzugsweise wobei das Organosulfid 2,5-Dimercapto-1,3,4-thiadiazol umfasst.

13. Verwendung einer Schmiermittelzusammensetzung zum Verbessern der Betriebstemperaturen eines Getriebes bei Hochlast- und Niedriggeschwindigkeitsbedingungen oder der Betriebseffizienz eines verwendeten Getriebes, wobei die Schmiermittelzusammensetzung umfasst:
a. ein Öl mit Schmierviskosität;
b. zu 0,5 bis 2,0 Gew.-% eine Aminalkyl(thio)phosphatverbindung und
c. zu 0,2 bis 0,8 Gew.-% ein Metallalkylthiophosphat, wobei das Schmiermittel einen Gesamtschwefelgehalt von 2 bis 5 Gew.-% umfasst.

## Revendications

1. Composition lubrifiante comprenant
a. une huile de viscosité lubrifiante ;
b. de 0, 5 à 2,0 % en poids d'un composé alkyl(thio)phosphate d'amine, et
c. de 0, 2 à 0,8 % en poids d'un alkylthiophosphate métallique,
dans laquelle la composition lubrifiante comprend une teneur totale en soufre de 2 à 5 % en poids.

2. Composition lubrifiante selon la revendication 1, dans laquelle l'alkyle(thio)phosphate d'amine comprend un phosphate d'amine.

3. Composition lubrifiante selon la revendication 2, dans laquelle le phosphate d'amine comprend un sel d'amine d'alkyle-phosphate essentiellement exempt de soufre dans lequel au moins 30 pour cent en moles des atomes de phosphore sont dans une structure de sel d'alkyl-pyrophosphate et au moins 80 pour cent en moles des groupes alkyle sont des groupes alkyle secondaires de 3 à 12 atomes de carbone ; ou dans laquelle le phosphate d'amine comprend un sel d'amine d'alkyle-phosphate essentiellement exempt de soufre dans lequel au moins 30 pour cent en moles des atomes de phosphore sont dans une structure de sel d'alkyle-pyrophosphate et au moins 25 pour cent en moles des groupes alkyle dans un tel alkyle-phosphate exempt de soufre sont des groupes alkyle primaires de 3 à 12 atomes de carbone.

4. Composition lubrifiante selon l'une quelconque des revendications précédentes, dans laquelle l'amine comprend du 2-éthylhexylamine.

5. Composition lubrifiante selon l'une quelconque des revendications précédentes, dans laquelle l'amine comprend un γ- ou δ-amino(thio)ester à substituant N-hydrocarbyle.

6. Composition lubrifiante selon la revendication 1 ou 2, dans laquelle l'alkyl(thio)phosphate d'amine comprend un alkylthiophosphate d'amine.

7. Composition lubrifiante selon la revendication 6, dans laquelle l'alkylthiophosphate de l'alkylthiophosphate d'amine comprend un dialkyldithiophosphate.

8. Composition lubrifiante selon la revendication 6 ou 7, dans laquelle l'amine comprend une alkylamine en C₈ à C₂₀.

9. Composition lubrifiante selon l'une quelconque des revendications précédentes, dans laquelle la composition comprend en outre du dialkyldithiophosphate de zinc.

10. Composition lubrifiante selon la revendication 9, dans laquelle le dialkyldithiophosphate de zinc comprend, est constitué essentiellement de, ou est constitué d'un dialkyldithiophosphate de zinc secondaire, de préférence dans laquelle l'alkyle du dialkyldithiophosphate de zinc comprend de 3 à 6 atomes de carbone.

11. Composition lubrifiante selon la revendication 9 ou 10, dans laquelle le dialkyldithiophosphate de zinc fournit de 0,02 à 0,095 % en poids de zinc à la composition lubrifiante.

12. Composition lubrifiante selon l'une quelconque des revendications précédentes, comprenant en outre moins de 6 % en poids d'un organosulfure, de préférence dans laquelle l'organosulfure comprend du 2,5-dimercapto-1,3,4-thiadiazole.

13. Utilisation d'une composition lubrifiante pour améliorer les températures de fonctionnement d'un engrenage à des conditions de charge basse et de vitesse élevée, ou l'efficacité de fonctionnement d'un engrenage utilisé, la composition lubrifiante comprenant :
a. une huile de viscosité lubrifiante ;
b. de 0, 5 à 2,0 % en poids d'un composé alkyl(thio)phosphate d'amine, et
c. de 0, 2 à 0,8 % en poids d'un alkylthiophosphate métallique, le lubrifiant comprenant une teneur totale en soufre de 2 à 5 % en poids.
